

**[54] NICKEL-CHROMIUM ALLOYS**

[76] Inventor: Miles Firnhaber, Rte. 3, Pewaukee, Wis. 53072

[21] Appl. No.: 896,701

[22] Filed: Apr. 17, 1978

[51] Int. Cl.<sup>2</sup> ..... C22C 19/05

[52] U.S. Cl. ..... 75/134 C; 75/171

[58] Field of Search ..... 75/171, 170, 134 C,  
75/134 F, 122; 148/32, 32.5

**[56] References Cited****U.S. PATENT DOCUMENTS**

3,876,423 4/1975 Firnhaber ..... 75/171

Primary Examiner—R. Dean

*Attorney, Agent, or Firm*—Fred Wiviot

**ABSTRACT**

A nickel-chromium alloy composed of the following ingredients in the following ranges of percentage by weight:

|    |       |   |       |
|----|-------|---|-------|
| Ni | 47.00 | — | 50.00 |
| Cr | 34.00 | — | 40.00 |
| Cu | .05   | — | .08   |
| Fe | 3.00  | — | 6.00  |
| C  | .18   | — | .30   |
| Si | .75   | — | 1.50  |
| Mn | .10   | — | .30   |
| Co | .75   | — | 1.50  |
| Mo | 2.50  | — | 3.50  |

2 Claims, No Drawings

## NICKEL-CHROMIUM ALLOYS

## BACKGROUND OF THE INVENTION

This invention relates to improvements in nickel-chromium alloys. 5

In centrifuges which are used in the manufacture of glass wool, the metal from which the centrifuge is formed must be resistant to attacks by molten glass which is high in borax and soda ash. In addition, it is 10 desirable in centrifuges or rotors of this type to have a multiplicity of relatively small peripheral holes from which the molten glass is thrown by centrifugal force into the path of fiberizing jets. The alloy, therefore, must be readily machinable. A rotor of this type is disclosed in Patent No. 3,227,536 and in my co-pending application Ser. No. 857,126, filed Dec. 5, 1977. Holes in centrifuges of this type are, of course, subject to wear and it is highly desirable to be able to provide a centrifuge which can be used for a maximum number of hours before there is objectionable wear on the holes. Another problem with metal centrifuges is that in the larger sizes there is a problem of distortion in use. Further, such 15 centrifuges are preferably corrosion resistant and can be operated at relatively high temperatures.

## SUMMARY OF THE INVENTION

It is a general object of the present invention to provide an improved nickel-chromium alloy which is particularly suitable for use in forming centrifuges useful in 30 the manufacture of glass wool.

A further object of the invention is to provide an alloy which is highly resistant to attack by the borax 35 and soda ash present in molten glass.

A further object of the invention is to provide an improved alloy which makes it possible to form a distortion free centrifuge in a diameter as large as 12".

A further object of the invention is to provide an 40 improved alloy, particularly adapted for use in centrifuges, which permits said centrifuge to be operated at a temperature as high as 2200° F. for a period as long as 2 hours without major deformation.

With the above and other objects in view the invention consists of the improved nickel-chromium alloy as set forth in the claims.

Centrifuges formed by the alloy of the present invention have been found to have superior corrosion resistance and high temperature strength than centrifuges formed by the alloy of U.S. Pat. No. 3,876,423.

## DESCRIPTION OF THE PREFERRED EMBODIMENT

The nickel-chromium alloy of the present invention is composed of the following ingredients in the following percentage ranges by weight:

|    |       |   |       |
|----|-------|---|-------|
| Ni | 47.00 | - | 57.00 |
| Cr | 34.00 | - | 40.00 |
| Cu | .05   | - | .08   |
| Fe | 3.00  | - | 6.0   |
| C  | .18   | - | .30   |
| Si | .75   | - | 1.50  |
| Mn | .10   | - | .30   |
| Co | .75   | - | 1.50  |

-continued

|    | Mo | 2.50  | - | 3.50 |
|----|----|-------|---|------|
| Ni |    | 54.00 |   |      |
| Cr |    | 35.00 |   |      |
| Cu |    | .05   |   |      |
| Fe |    | 4.50  |   |      |
| C  |    | .27   |   |      |
| Si |    | 1.00  |   |      |
| Mn |    | .20   |   |      |
| Co |    | 1.10  |   |      |
| Mo |    | 3.00  |   |      |

The preferred formula is as follows:

15 For preparation, any of the conventional procedures for nickel alloys may be followed. For example, the nickel and chromium are melted in an electric arc furnace at a temperature of about 2800°-3000° F. The other alloying elements are then added and the temperature raised to 20 promote homogeneity.

25 Centrifuges manufactured by an alloy as above described were used in the manufacture of glass fibers and the centrifuges were found to stand up for an exceptionally long time against corrosive effects of glass batches which were high in borax and soda ash. Centrifuges made with alloys in accordance with the present invention were also found to have superior high temperature strength and creep resistance and is readily machinable.

Various changes and modifications may be made in the invention heretofore described as may be within the scope of the claims.

I claim:

1. An alloy consisting of the following ingredients in percentages by weight:

|    |       |   |       |
|----|-------|---|-------|
| Ni | 47.00 | - | 57.00 |
| Cr | 34.00 | - | 40.00 |
| Cu | .05   | - | .08   |
| Fe | 3.00  | - | 6.0   |
| C  | .18   | - | .30   |
| Si | .75   | - | 1.50  |
| Mn | .10   | - | .30   |
| Co | .75   | - | 1.50  |
| Mo | 2.50  | - | 3.50  |

45 said alloy being characterized by resistance to corrosive attack by molten glass, having superior creep resistance, having strength at elevated temperatures, and imparting resistance to deformation to articles made therefrom.

2. An alloy in which the ingredients are in about the 50 following percentages by weight:

|    |       |  |  |
|----|-------|--|--|
| Ni | 54.00 |  |  |
| Cr | 35.00 |  |  |
| Cu | .05   |  |  |
| Fe | 4.50  |  |  |
| C  | .27   |  |  |
| Si | 1.00  |  |  |
| Mn | .20   |  |  |
| Co | 1.10  |  |  |
| Mo | 3.00  |  |  |

60 said alloy being characterized by resistance to corrosive attack by molten glass, having superior creep resistance, having strength at elevated temperatures, and imparting resistance to deformation to articles made therefrom and resistance to cracking after prolonged exposure to elevated temperatures above 2000° F.

\* \* \* \* \*